

## UNITED STATES PATENT OFFICE

2,525,078

## METAL CLEANING COMPOSITION

Arthur C. Pabst, Douglaston, and Eleanor S. Salmon, New York, N. Y., assignors to Socony-Vacuum Oil Company, Incorporated, a corporation of New York

No Drawing. Application October 8, 1947,  
Serial No. 778,732

8 Claims. (Cl. 252—143)

1

This invention relates to improved metal cleaning compositions and their use. It is particularly directed to metal cleaning compositions capable of removing rust, scale, grease and other deposits from metal surfaces.

One of the main uses for such a composition is in the cleaning of water cooling systems such as are used in internal combustion engines. Such systems gradually become fouled during use and unless periodically shut down and cleaned, the water jackets and radiators become coated with deposits which interfere with the heat transfer and in severe cases may be plugged to a point of complete stoppage of coolant circulation. The composition of the deposits may vary depending upon the construction materials of the coolant system. Such metals as solder, copper, zinc, lead and iron may be used in one form or another and, of these, iron in its various modifications is the chief component. Grease may enter the cooling system from grease packed water pumps and oil or oxidized hydrocarbons may enter from "blow-by" from the combustion chamber or from other sources. Certain other foreign deposits may be introduced with the coolant especially when it is water. A common component of the fouling deposits is iron oxide cemented fast to the metal surface by adsorbed or oxidized oil. Such a scale especially when covered with a coating of grease or oil is very difficult to remove.

Similar conditions prevail and similar contaminants consisting of oxidized metal and oily substances are usually present on the surfaces of machine parts which are to be cleaned in shops. The cleaning operations usually comprise degreasing, pickling and de-rusting.

Cleaning compositions used at present for automotive cooling systems may be generally classified under one of three types. One type consists of an aqueous solution of an alkaline salt such as washing soda, trisodium phosphate, etc. This type acts very slowly on rust and scale so that only small amounts of the deposits are removed in the time normally given the radiator flushing. Moreover, it removes very little of the oil or grease deposits. A second type of cleaner consists of an alkaline emulsion of hydrocarbons and other organic solvents. This type will remove the oil and grease deposits fairly satisfactorily but will remove only very small amounts of rust and scale deposit; consequently, the system is not entirely cleaned. The third type of cleaner consists of aqueous solutions of acids or acid salts, such as hydrochloric and oxalic acids and sodium bisulfate. This type is very effective in removing rust and scale but will

2

remove very little grease or oil deposit. Moreover, the acid type cleaner is highly corrosive and requires a "follow-up" flush with an alkali to stop the action of the acid. This is not always satisfactory in entirely avoiding corrosion as it is often difficult to obtain complete acid neutralization.

A major object of this invention is the provision of a new and novel cleaning composition which is capable of removing rust, scale and oily deposits.

A further object of this invention is the provision of a cleaning composition which will rapidly remove rust and scale deposits from metal surfaces without causing rapid "after corrosion" of the metal surface.

Another object is the provision of a rapid method for cleaning metal surfaces and cooling systems which will not cause considerable surface corrosion. These and other objects will become apparent from the more detailed description of the invention following hereinafter.

We have now discovered that certain oil-in-acid solution type emulsions will rapidly remove rust and scale from metal surfaces and at the same time dissolve and emulsify any oil and grease present. Tests also indicate that the product has remarkable properties in inhibiting corrosion so that it is unnecessary to follow up with an alkaline wash. In other words, the product offers the main advantages of each of the types of common radiator flushes without their disadvantages and failings. Moreover, the product of this invention may be packaged in concentrated form and will remain stable and substantially unchanged after long periods of storage. Thus the product in a very small container may be stored on a shelf for a period of months and then when needed it may be readily diluted in water to provide a cleaning emulsion of the desired strength for cleaning metal surfaces such as in automobile radiators.

The cleaning composition of this invention consists of a dispersed phase of an emulsifiable organic water-insoluble material and a continuous phase of a strong aqueous solution of hydrochloric acid, and a specific emulsifying agent capable of producing emulsions sufficiently stable both for long shelf storage prior to use and for subsequent dilution if desired at the time of use while still forming a stable emulsion. The continuous phase should consist of an aqueous solution of hydrochloric acid in which the concentration of pure HCl is within the range 10-30 percent by weight and preferably within the range 15-25 percent by weight. It is by virtue

of these high acid concentrations that the cleaning composition can be prepared long periods before it is to be actually used and packaged in relatively small bulk as compared with the bulk of the diluted cleaning emulsion which is actually finally employed for cleaning the automobile radiator. The dispersed phase may consist either of hydrocarbon solvents or of halogenated hydrocarbon solvents or mixtures thereof; exemplary are kerosene and orthodichlorbenzene. Halogenated hydrocarbons either alone or in admixture with straight hydrocarbons are particularly desirable as they tend to form stable emulsions more readily. Such hydrocarbons and halogenated hydrocarbons should boil above about 160° F. in order to prevent loss thereof by evaporation during use. Preferably the halogenated hydrocarbons and particularly the hydrocarbons should boil above about 250° F.

The emulsifier to be used is one capable of 20

5 mol of beta-hydroxyethyl ethylene diamine with 0.5 mol of commercial oleic acid and then heating under reflux for about 5 hours until a final temperature of about 507° F. is reached. During this period about 2 mols of water per mol of oleic acid are distilled off. Excess hydroxyethyl ethylene diamine is then removed and the product, 1-hydroxyethyl 2-heptadecenyl glyoxalidine is purified by vacuum distillation. We have 10 found it preferable to employ mixtures of 1-hydroxyethyl 2-heptadecenyl glyoxalidine and an iso-octyl phenyl polyglycol ether of about 650 molecular weight in our cleaning composition. Mixtures of these emulsifiers have been found 15 to result in even more stable oil in acid emulsions than compositions employing only one of the emulsifiers.

The following examples will illustrate the type 15 of emulsions made and used according to this invention.

| Emulsion No.                                                                                    | I                  | II                 | III                | IV                 | V                  | VI                 | VII                | VIII               | IX                 | X                  |
|-------------------------------------------------------------------------------------------------|--------------------|--------------------|--------------------|--------------------|--------------------|--------------------|--------------------|--------------------|--------------------|--------------------|
| Constituents                                                                                    | Weight<br>Per cent | Weight<br>Per cent | Weight<br>Per cent | Weight<br>Per cent | Weight<br>Per cent | Weight<br>Per cent | Weight<br>Per cent | Weight<br>Per cent | Weight<br>Per cent | Weight<br>Per cent |
| Orthodichlorbenzene                                                                             | 20.0               | 20.0               | 20.0               | 39.5               | 19.5               | 19.0               | 30.0               | 30.0               | 15.0               | 20.0               |
| Carbon Tetrachloride                                                                            |                    |                    |                    |                    |                    |                    |                    |                    |                    |                    |
| Kerosene                                                                                        | 20.0               | 19.5               | 19.5               |                    | 19.0               | 19.5               | 30.0               | 30.0               | 15.0               | 20.0               |
| Naphtha (250-450° F. boiling range)                                                             |                    |                    |                    |                    |                    |                    |                    |                    |                    |                    |
| Concentrated HCl (38%)                                                                          | 58.5               | 27.0               | 27.0               | 59.0               | 27.0               | 16.9               | 15.9               | 15.9               | 27.0               |                    |
| 1-hydroxyethyl 2-heptadecenyl glyoxalidine                                                      | 1.5                | 1.5                |                    | 5.0                | 1.5                | 1.5                | 5.0                |                    |                    |                    |
| Para-iso-octyl polyglycol phenyl ether (10 mols glycol per mol of iso-octyl phenol M. W. @ 650) |                    |                    |                    |                    |                    |                    |                    |                    |                    |                    |
| Water                                                                                           |                    |                    |                    |                    | 1.5                | 1.0                | 1.0                | 5.0                | 1.5                | 3.0                |
|                                                                                                 |                    | 32.0               | 32.0               | 28.5               |                    | 32.0               | 49.1               | 49.1               | 52.6               | 30.0               |

giving either a completely stable emulsion or a readily redispersable product when the emulsion is stored over long periods of time, for example as shelf goods. We have found that a stable oil in strong hydrochloric acid solution emulsion may be provided when our cleaning composition contains as an emulsifier a compound which may be expressed by the formula



where R is a di-isobutyl phenyl radical and n is a number between about 6 and 15 and preferably equal to about 10. This emulsifier may be referred to generically as iso-octyl phenyl polyglycol ether or polyethylene glycol mono iso-octyl phenyl ether. This emulsifier may be prepared as described in the following example:

206 parts of para-iso-octyl phenol (obtainable by condensing phenol with di-iso-butylene by known methods) are melted and 2 parts of a caustic soda solution of 40 percent strength are added thereto. Ethylene oxide is introduced, while stirring at a temperature of 248 to 267° C. until 10 mols of ethylene oxide per one mol of para-iso-octyl phenol have been absorbed. The resulting product is a para-iso-octyl phenyl polyglycol ether having a polyglycol radical consisting of 10 molecular proportions of glycol and a total molecular weight of about 646.

Using the same method described above but limiting the amount of ethylene oxide absorbed to about six mols per mol of iso-octyl phenol an emulsifier having a molecular weight of about 470 may be obtained. While it is preferred that the iso-octyl phenyl polyglycol ether employed have a molecular weight of about 650, still in less preferred forms of this invention it may vary in molecular weight within the range about 470 to 875.

Another emulsifier which may be employed is 1-hydroxyethyl 2-heptadecenyl glyoxalidine. This compound may be prepared by mixing one

35 5 mol of beta-hydroxyethyl ethylene diamine with 0.5 mol of commercial oleic acid and then heating under reflux for about 5 hours until a final temperature of about 507° F. is reached. During this period about 2 mols of water per mol of oleic acid are distilled off. Excess hydroxyethyl ethylene diamine is then removed and the product, 1-hydroxyethyl 2-heptadecenyl glyoxalidine is purified by vacuum distillation. We have 10 found it preferable to employ mixtures of 1-hydroxyethyl 2-heptadecenyl glyoxalidine and an iso-octyl phenyl polyglycol ether of about 650 molecular weight in our cleaning composition. Mixtures of these emulsifiers have been found 15 to result in even more stable oil in acid emulsions than compositions employing only one of the emulsifiers.

The following examples will illustrate the type 15 of emulsions made and used according to this invention.

These emulsions are prepared by dissolving the emulsifier in one of the phases, generally the one in which the emulsifier is most soluble, and then adding the other liquid phase while stirring the liquid with a high speed mixer. The hydrocarbon emulsion in aqueous acid thus formed may be further diluted with water, if desired. Either the cationic emulsifier 1-hydroxyethyl 2-heptadecenyl glyoxalidine or the non-ionic emulsifier, polyethylene-glycol mono iso-octyl phenyl ether are soluble in the oil phase and may be dissolved therein and the acid then added. Moreover, the former emulsifier is also soluble in aqueous acid solution, so that it may first be dissolved therein and the oil phase added with mixing. The desirable amount of emulsifier to be used may vary between 0.1% to 5.0% by weight of the emulsion. In use the prepared emulsion may be added to the cooling system or to a circulating bath in concentrations controlled to provide the desired cleaning rate. Thus, for example, such prepared emulsions as shown in the above table may be added to water in a cooling system in concentrations of 5% emulsion and upwards. In any event the pH value of the liquid circulated in the cleaning system should be below 4.0, and the acid concentration in the continuous phase should be of the order of about 1.0% by weight HCl, and upwards.

After the emulsion is added to the cooling system or cleaning bath, it is heated either by a heater or by starting the engine involved and the heated emulsion is circulated. After about 20 to 30 minutes of circulation, the system is drained and flushed by filling with water and running the engine until warm. The water is then drained and the system refilled with cooling water. After such a treatment, the metal surfaces of the cooling system are thoroughly clean of rust, scale, water deposits and grease. When the cleaning solution is used for cleaning metal parts or tools, the parts or tools are placed in a

bath of the emulsion for a set period, then removed and rinsed in clean water. No neutralizing chemicals need be added to the rinsing water to prevent corrosion of the metal cleaned.

In addition to the practical tests on automobile cooling systems, as described hereinabove, laboratory tests were also made to establish the relative cleaning efficiencies of these novel emulsions and of certain cleaning compositions used commercially heretofore. Rusted steel plates were immersed in the boiling solutions in concentrations recommended by the respective manufacturers, and the time required for completion of cleaning was taken as a measure of efficiency. The after corrosion of the metal was particularly noted.

| Cleaning Compound                                    | Concentration of Active Acid or Salt in Cleaning Bath | Time, in minutes, to complete cleaning | After-corrosion in four days |
|------------------------------------------------------|-------------------------------------------------------|----------------------------------------|------------------------------|
| Oxalic Acid type                                     | Gm./liter                                             | 30                                     | noticeable.                  |
| Sodium bisulfate type                                | 20                                                    | 30                                     | Do.                          |
| Hydrochloric acid type                               | 23                                                    | 7                                      | strong.                      |
| Emulsion II (1 part emulsion II to 9 parts of water) | 10                                                    | 7                                      | none.                        |

It will be apparent from the above that the emulsions of this invention have substantially the same rust removing power as strong acid type commercial cleaning compositions while at the same time protecting the metal surface cleaned from after corrosion. Moreover, the emulsions have a far greater grease and oil removing power than the acid or acid salt type cleaning compo-

sitions. The stable hydrocarbon-in-acidic-solution emulsion permits a uniformity of hydrocarbon distribution throughout the cleaning solution so that it may perform its function uniformly over the entire surface of the metal to be cleaned.

To further prove that the emulsion type cleaning compositions of this invention are less corrosive on the metal surfaces or cooling systems being cleaned, even while being used, a number of uniform strips of the metals commonly encountered in cooling systems were immersed in several different cleaning liquids for a period of 24 hours and the corrosion loss was then measured.

15

| Cleaning Compound      | Concentration of Active Acid or Salt in Cleaning Bath | Corrosion loss at 160° F. in 24 hours |             |
|------------------------|-------------------------------------------------------|---------------------------------------|-------------|
|                        |                                                       | Iron                                  | Solder      |
| Oxalic Acid type       | Gm./liter                                             | Milli-grams                           | Milli-grams |
| Hydrochloric Acid type | 20                                                    | 146                                   | 33.5        |
| Emulsion II (1:9)      | 23                                                    | 3,149                                 | 748         |
| Sodium bisulfate type  | 10                                                    | 52                                    | 19.1        |
|                        | 20                                                    | 300                                   | 21.1        |

It should be understood that the specific examples of the emulsion type cleaning compositions and of their application as given hereinabove are intended merely as exemplary and are not to be construed as limiting the scope of this invention thereto. These compositions present a very considerable and useful stability over related compositions known to the prior art as may be seen from the following data.

#### Acid emulsions—Metal cleaning compounds

|                                                               | 1     | 2     | 3     | 4     | 5     | 6     | 7     | 8     | 9    | 10   | 11    | 12    | 13    | 14    |
|---------------------------------------------------------------|-------|-------|-------|-------|-------|-------|-------|-------|------|------|-------|-------|-------|-------|
| Concentrated HCl (38%)                                        | 59.0  | 59.0  | 59.0  | 59.0  | 59.0  | 59.0  | 59.0  | 15.9  | 15.9 | 15.9 | 27.0  | 15.9  | 15.9  | 15.9  |
| Hydrocarbon solvents of kerosene boiling range                | 19.0  | 19.5  | 17.5  | 19.5  | 19.5  | 19.5  | 19.5  | 30.0  | 30.0 | 30.0 | 19.0  | 30.0  | 30.0  | 15.0  |
| Orthodichlorbenzene                                           | 19.5  | 20.0  | 18.5  | 20.0  | 20.0  | 20.0  | 20.0  | —     | —    | —    | 19.5  | —     | —     | 15.0  |
| 1-hydroxyethyl, 2-heptadecenyl, glyoxalidine.                 | 1.5   | —     | —     | —     | —     | —     | —     | —     | —    | —    | 1.5   | 5.0   | —     | —     |
| Polyethylene-glycol mono iso-octyl phenyl ether <sup>12</sup> | 1.0   | —     | —     | —     | —     | —     | —     | —     | —    | —    | 1.0   | —     | 5.0   | 1.5   |
| Olef. Acid                                                    | —     | —     | —     | —     | —     | —     | —     | 5.0   | —    | —    | —     | —     | —     | —     |
| Sodium Lauryl Sulfate                                         | —     | 1.5   | 5.0   | —     | —     | —     | —     | —     | —    | —    | —     | —     | —     | —     |
| Gum Tragacanth                                                | —     | —     | —     | 1.5   | —     | —     | —     | —     | —    | —    | —     | —     | —     | —     |
| Polyethylene Glycol Monoleate 600                             | —     | —     | —     | —     | 1.5   | —     | —     | —     | —    | —    | —     | —     | —     | —     |
| Polyethylene Glycol Dioleate 600                              | —     | —     | —     | —     | —     | 1.5   | —     | —     | —    | —    | —     | —     | —     | —     |
| Polyethylene Glycol Oleate 400L                               | —     | —     | —     | —     | —     | —     | 1.5   | —     | —    | —    | —     | —     | —     | —     |
| Polyethylene Glycol 1000 mono-oleate                          | —     | —     | —     | —     | —     | —     | —     | 5.0   | 5.0  | 5.0  | —     | —     | —     | —     |
| Polyethylene Glycol 1000 di-oleate                            | —     | —     | —     | —     | —     | —     | —     | 10.0  | 10.0 | 10.0 | —     | —     | —     | —     |
| Polyethylene Glycol 4000 di-oleate                            | —     | —     | —     | —     | —     | —     | —     | —     | 10.0 | —    | —     | —     | —     | —     |
| Water                                                         | —     | —     | —     | —     | —     | —     | —     | 34.1  | 34.1 | 34.1 | 32.0  | 49.1  | 49.1  | 52.6  |
|                                                               | 100.0 | 100.0 | 100.0 | 100.0 | 100.0 | 100.0 | 100.0 | 100.0 | 95.0 | 95.0 | 100.0 | 100.0 | 100.0 | 100.0 |
|                                                               | (1)   | (2)   | (3)   | (4)   | (5)   | (6)   | (7)   | (8)   | (9)  | (10) | (11)  | (12)  | (13)  | (14)  |

<sup>1</sup> Emulsion stable for 1 day. Separates into 2 emulsion layers in 3 days. Redispersed by simple shaking after 6 months. Forms stable emulsion when diluted, can be boiled.

<sup>2</sup> Unstable. Total Separation and no redispersion after 5-10 minutes.

<sup>3</sup> Unstable. Separation begins within 5-10 minutes. Total separation and no redispersion after 12 hours.

<sup>4</sup> No emulsion. Water phase too thick. Cannot be dispersed.

<sup>5</sup> Stable for 1 day. Separates into 2 clear phases in 3 days and cannot be redispersed by vigorous shaking. Cannot be diluted. Forms no emulsion in water.

<sup>6</sup> Stable for 1 day. Separates into 2 clear phases in 3 days and cannot be redispersed by vigorous shaking. Cannot be diluted. Forms no emulsion in water.

<sup>7</sup> Stable for 1 day. Separates into 2 clear phases in 3 days and cannot be redispersed by vigorous shaking. Cannot be diluted. Forms no emulsion in water.

<sup>8</sup> Emulsion separates into 2 opaque layers overnight. May be redispersed by mild agitation. After 4 days separates into 2 layers which cannot be recombined by vigorous agitation. No longer completely disperses in water.

<sup>9</sup> Separates into 2 layers over-night which recombine by mild agitation. After 4 days separates into clear oil layer and opaque layer cannot be redispersed by shaking. No longer completely disperses in water.

<sup>10</sup> Separates permanently on standing over-night into one clear oil layer and an opaque layer. Cannot be redispersed by shaking. No longer disperses completely in water.

<sup>11</sup> Separates into 2 emulsion layers in 3 days which may be redispersed by simple shaking. After 6 months separates into 2 emulsion layers which may be redispersed by simple shaking. After 6 months still forms stable emulsion when diluted. Can be boiled.

<sup>12</sup> After 65 days storage separates into 2 emulsion layers and a very slight water layer which may be redispersed by simple shaking. After 65 days still forms stable emulsion when diluted with water.

<sup>13</sup> After 75 days storage separates into 2 emulsion layers and a very slight water layer which may be redispersed by simple shaking. After 75 days still forms stable emulsion when diluted with water.

<sup>14</sup> After 75 days storage separates into 2 emulsion layers and a very slight water layer which may be redispersed by simple shaking. After 75 days still forms stable emulsion when diluted with water.

<sup>15</sup> M. W. @ 650—i. e., containing about 10 molecular portions of (CH<sub>2</sub>CH<sub>2</sub>O).

In the above table compositions numbered 1, 11, 12, 13 and 14 are compositions prepared according to the instant invention, compositions 1 and 11 representing the preferred form of the invention. Compositions 2 and 3 employ an emulsifier which has been used in the prior art in preparing oxalic acid emulsions. Compositions 4-10 are typical of the emulsions shown in United States Patent 2,269,529 issued January 13, 1942, to Goldsmith. It will be seen that the compositions prepared according to the method of this invention are stable in that after long periods of standing no clear oil layer separates and the emulsion layers which do separate may be redispersed by simple shaking to provide an emulsion having substantially the same appearance and properties as the composition when originally made. Moreover, the cleaning compositions of this invention after long periods of standing (65 days—6 months and upwards) can be diluted with water to form a completely dispersed stable emulsion. This dilute emulsion can be boiled without destruction of the emulsion. It will be noted that in the case of compositions 2-10, upon standing from one to six days, a clear oil layer separates out indicating complete break down of the emulsion. The separated layers in the latter compositions cannot be redispersed even on vigorous shaking and cannot be dispersed completely in water upon dilution. It will be apparent that in the case of compositions 2-10, these compositions cannot be employed for cleaning metals or automobile radiators after having been stored for any appreciable time without danger of severe corrosion of the metal surfaces due to the acid. The compositions of the instant invention on the other hand being stable emulsions do not involve this critical difficulty.

This case is a continuation in part of our application Serial Number 616,479, filed September 14, 1945 (now abandoned), which is in turn a continuation in part of our application Serial Number 562,902, filed November 10, 1944 now abandoned.

We claim:

1. A metal cleaning composition in the form of an oil-in-water emulsion which comprises, a dispersed phase of a substantially water-insoluble organic solvent selected from the group consisting of kerosene, naphtha boiling within the range about 250° F. to 450° F. and liquid chlorinated hydrocarbons boiling above about 160° F. and mixtures of the same, a continuous phase of an aqueous solution of hydrochloric acid in which the percentage by weight HCl is within the range 15 to 25, and about 0.1 percent to about 5.0 percent by weight of the emulsion of iso-octyl phenyl polyglycol ether having a molecular weight of about 650 as an emulsifier.

2. A metal cleaning composition in the form of an oil-in-water emulsion which comprises, a dispersed phase of a substantially water-insoluble organic solvent selected from the group consisting of kerosene, naphtha boiling within the range about 250-450° F., liquid chlorinated hydrocarbon boiling above about 160° F. and mixtures of the same, a continuous phase of an aqueous solution of hydrochloric acid containing about 10 to 30 percent by weight HCl and about 0.1 to 5.0 percent by weight of the emulsion of an emulsifier which is the product of the general formula:



wherein R stands for a di-iso-butyl phenyl radical and n stands for a whole number from 6-15.

3. A metal cleaning composition in the form of an oil-in-water type emulsion which comprises, a dispersed phase of an emulsifiable organic water-insoluble solvent selected from the group consisting of kerosene, naphtha boiling within the range about 250° F.-450° F., liquid chlorinated hydrocarbons boiling above about 160° F. and mixtures of the same, a continuous phase of an aqueous solution of hydrochloric acid in which the concentration of HCl is within the range about 10 to 30 percent by weight and about 0.1 to 5.0 percent by weight of the emulsion of an emulsifier consisting of a mixture of 1-hydroxyethyl 2-heptadecenyl glyoxalidine and iso-octyl phenyl polyglycol ether having a molecular weight within in the range about 470-875.

4. A metal cleaning composition in the form of an oil-in-water type emulsion which comprises, a dispersed phase of a solvent selected from the group consisting of kerosene, naphtha boiling within the range about 250° F.-450° F., liquid chlorinated hydrocarbons boiling above about 160° F. and mixtures of the same, a continuous phase of an aqueous solution of hydrochloric acid in which the concentration of HCl is within the range about 10 to 30 percent by weight and about 0.1 to 5.0 percent by weight of the emulsion of an emulsifier consisting of a mixture of 1-hydroxyethyl 2-heptadecenyl glyoxalidine and the product of the general formula



wherein R stands for a di-isobutyl phenyl radical.

5. A metal cleaning composition in the form of an oil-in-water type emulsion which comprises, a dispersed phase consisting of a mixture of kerosene and orthodichlorbenzene, a continuous phase of an aqueous solution of hydrochloric acid in which the concentration of HCl is within the range about 10 to 30 percent by weight and about 0.1 to 5.0 percent by weight of the emulsion of an emulsifier consisting of a mixture of 1-hydroxyethyl 2-heptadecenyl glyoxalidine and the product of the general formula



wherein R stands for a di-isobutyl phenyl radical.

6. A metal cleaning composition in the form of an oil-in-water type emulsion which comprises, a dispersed phase of a mixture of a hydrocarbon solvent fraction boiling above about 250° F. and not above about 450° F. and orthodichlorbenzene, a continuous phase of an aqueous solution of hydrochloric acid in which the concentration of HCl is within the range about 10-30 percent by weight, and about 0.1-5.0 percent by weight of the emulsion of an emulsifier which is a compound having the formula



wherein R stands for a di-isobutyl phenyl radical and n stands for a whole number within the range 6-15.

7. A metal cleaning composition in the form of an oil-in-water type emulsion which comprises, a dispersed phase of a mixture of a naphtha boiling within the range about 250° F.-450° F. and carbon tetrachloride, a continuous phase of an aqueous solution of hydrochloric acid in which the concentration of HCl is within the range about 10-30 percent, and about 0.1 to 5.0 percent by weight of the emulsion of an emulsifier which is a compound having the formula



## REFERENCES CITED

The following references are of record in the file of this patent:

## UNITED STATES PATENTS

| Number       | Name            | Date          |
|--------------|-----------------|---------------|
| 2,036,848    | Amthor -----    | Apr. 7, 1936  |
| 2,261,700    | Ryznar -----    | Nov. 4, 1941  |
| 2,269,529    | Goldsmith ----- | Jan. 13, 1942 |
| 10 2,302,697 | Katzman -----   | Nov. 24, 1942 |
| 2,396,776    | Douty -----     | Mar. 19, 1946 |
| 2,399,205    | Campbell -----  | Apr. 30, 1946 |
| 2,399,267    | Szatyn -----    | Apr. 30, 1946 |

wherein R stands for a di-isobutyl phenyl radical and n stands for a whole number within the range 6-18.

8. A metal cleaning composition in the form of an oil-in-water type emulsion which comprises a dispersed phase consisting of kerosene, a continuous phase of an aqueous solution of hydrochloric acid in which the concentration of HCl is within the range about 10-30 percent by weight and about 0.1 to 5.0 percent by weight of the emulsion of an emulsifier consisting of a mixture of polyethylene glycol mono iso-octyl phenyl ether and 1-hydroxyethyl 2-heptadecenyl glyoxalidine.

ARTHUR C. PABST.

ELEANOR S. SALMON. 15